

**1**

3,843,538

**DEVELOPING EMULSION FOR ELECTROSTATIC IMAGES**

Marinus Cornelius Vermeulen, Valley View, Ian Edward Smith, Lockleys, and Peter John Hastwell, North Adelaide, Australia, assignors to Savin Business Machines Corporation, Valhalla, N.Y.  
No Drawing. Filed July 7, 1972, Ser. No. 269,603  
Int. Cl. G03g 9/04

U.S. Cl. 252—62.1

4 Claims

**ABSTRACT OF THE DISCLOSURE**

An emulsion for developing electrostatic images comprising a disperse water phase and a continuous phase which is a solution of a pigmented high molecular weight polymer dissolved in an appropriate organic solvent. The emulsion is non-conductive, may be stabilized by a surface-active emulsifying agent which has a predetermined hydrophilic-lipophilic balance, and may include a protective colloid and a defoaming agent. If desired, a release agent may be employed in the continuous phase of the emulsion.

**BACKGROUND OF THE INVENTION**

In our co-pending application, Ser. No. 155,108, filed June 21, 1971, for "Method of Contact Transfer of Developed Electrostatic Images and Means for Practicing Same," we disclosed a developing liquid for developing a latent electrostatic image which comprised a solution of a high molecular weight resin substantially insoluble in a light hydrocarbon liquid, which solution is dispersed or suspended in such light hydrocarbon liquid. The light hydrocarbon liquid is adapted to be evaporated from a developed latent electrostatic image and to leave a tacky developed image on a photoconductive surface on which the latent electrostatic image is formed. The tacky image is adapted to be transferred to a sheet of paper or other sheet material by contact with the tacky image. After drying, the paper carries the final reproduction of the original. In order to assist in the transfer of the developed tacky toner image from the photoconductive surface to the paper surface, we disclosed that the photoconductive surface could be coated with a silicone or a urethane film in order to reduce the affinity of the tacky developed image for the photoconductor and thus assist in the ready transfer of the image to the paper surface.

In our co-pending application,<sup>1</sup> Ser. No. 269,054, filed July 5, 1972, for "Improved Developing Liquid for Electrostatic Images," we disclosed that a minor amount of release agent could be suspended in the carrier liquid. The release agent had to be insoluble in the carrier liquid and had to be of electrophoretic nature. It was taught that the carrier liquid had to be a light hydrocarbon since it must be non-conductive and so that it could evaporate readily to leave a diluent-free developed tacky image which could then be transferred. As the speed of operation of electrophotographic apparatus increases, more evaporated light hydrocarbons are discharged into the atmosphere tending to pollute it. The pollution problem becomes a serious one when one operates a machine using a light hydrocarbon liquid as a carrier at high speeds in closed areas.

We have succeeded in emulsifying a solution of an organosol with water, so that the diluent liquid is water which, when evaporated, will not pollute the atmosphere. When a latent electrostatic image is developed with our aqueous emulsion, the tacky toner is attracted to the charged portions, thus in effect breaking the emulsion

**2**

locally. The released water can be squeegeed or blown from the surface of the photoconductor and the tacky toner image may be transferred to the paper as described in our co-pending application, Ser. No. 155,108.

A pneumatic assembly for removing excess developer liquid from photoconductive surfaces is shown in our co-pending application, Ser. No. 200,433, filed Nov. 19, 1971, and now U.S. Pat. 3,741,643.

**Summary of the Invention**

One object of our invention is to provide an aqueous emulsion in which the oil phase comprises a solution of a tacky toner—that is, an organosol such as disclosed in our co-pending application, Ser. No. 155,108.

Another object of our invention is to provide an emulsion of a solution of a tacky toner and water, so that the pollution of the atmosphere caused by the evaporation of light hydrocarbons is substantially reduced.

Another object of our invention is to provide a stable emulsion in which the water phase is dispersed and in which the continuous phase is a solution of a pigmented high molecular weight polymer dissolved in an appropriate organic solvent.

Another object of our invention is to provide a developing emulsion of the W/O type. This can be employed with an organic photoconductive surface which is normally hydrophobic such as trinitro-fluorenone and polyvinyl carbazole coated on a conductive base such as vacuum-evaporated aluminum deposited on polyester film.

Another object of our invention is to provide an emulsion for developing latent electrostatic images formed on an inorganic photoconductive surface such as zinc oxide which has been coated with a hydrophobic layer such as silicone.

Another object of our invention is to provide an aqueous emulsion for developing latent electrostatic images having a predetermined hydrophilic-lipophilic balance, which is non-conductive and in which water is in the disperse phase.

Other and further objects of our invention will appear from the following description.

In general, the tacky or adhesive toner composition is the lipide component of the emulsion. It comprises a high molecular weight resin or mixture of high molecular weight resins dissolved in an organic solvent. In general the organic solvent comprises a light hydrocarbon liquid which includes about 90% isoparaffinic hydrocarbons and about 10% aromatic hydrocarbons. The aqueous or water phase comprises distilled water and a dispersing agent of the surface-active type. The emulsifying agent must be more soluble in or better wetted by the lipide phase than by the disperse or aqueous phase. A defoaming agent and a protective colloid may be added to the water phase. The emulsion may be formed in any appropriate manner, as by milling in a colloid mill, a homogenizer, or by sonic or ultrasonic equipment.

More particularly, a lipide component is formed as follows:

**EXAMPLE 1**

The following materials:

37.5 grams "PLIOLITE VTAC"  
40.0 grams "SOLPRENE 1205"  
100.0 grams "SOLVESSO 100"

are emulsified in a high-speed emulsifying mill together with 1000 grams of "ISOPAR G." "PLIOLITE VTAC" is a vinyl-toluene/acrylate copolymer manufactured by Goodyear Tire & Rubber Company, of Akron, Ohio. "SOLPRENE 1205" is a copolymer of butadiene and styrene in the ratio of 75/25, manufactured by the solution

<sup>1</sup> Attorneys' docket number: Smith *et al.* Case 53.

polymerization process, and sold by Phillips Petroleum Company. "ISOPAR G" is an isomerized paraffinic hydrocarbon having a specific gravity of .75 at 0° F. and is substantially 100% pure isoparaffinic hydrocarbon. It has a boiling range from 157° C. to 177° C. "SOLVESSO" is a hydrocarbon solvent manufactured by Standard Oil Company of New Jersey. It has an initial boiling point of 159° C. and a final boiling point or end point of 182° C. It comprises largely aromatic hydrocarbons and has a kauri-butanol number of 91.

A toner matching the organosol is then formed as follows. We take:

100.0 grams microlith black  
12.5 grams reflex blue  
25.0 grams "PLIOLITE VTAC"  
25.0 grams "SOLPRENE 1205"

and add sufficient toluol to achieve correct milling viscosity. This mixture is milled in a cavitation mill and 120 grams of the toner is added to the organosol circulating in the mill.

The aqueous phase is formed as follows:

125.0 grams of distilled water  
0.5 grams of an antifoam agent such as ethylene oxide condensate of stearic acid  
1.25 grams of starch (protective colloid).

The emulsion is then formed by taking 250 grams of this lipide component to which we add 7 grams of mineral turps and emulsify the lipide component with the aqueous component.

This is accomplished by milling the aqueous and lipide phases in a colloid mill for three minutes. This mill mix will produce images on a negatively charged photoconductor. The excess toner liquid is removed with a squeegee roller or by an air knife. When the image is formed, the emulsion is broken locally by the deposit of the lipide phase to form the desired reproduction. The water phase forms droplets on the background area. These water droplets are removed by an air knife and leave the background of the photoconductor completely dry. It is to be noted that an emulsifying or dispersing agent was not used in Example 1. The emulsion was employed shortly after it was formed. The defoamer was used mainly to counteract the aeration of the milling which is undesirable.

#### EXAMPLE 2

The following organosol was formed. We mixed:

37.5 grams "PLIOLITE VTAC"  
10.0 grams "SOLPRENE 1205"  
100.0 grams "SOLVESSO."

To this we added 240 grams of the toner component of Example 1 and 1000 grams of "ISOPAR G." These were milled in a colloid mill for three minutes.

The water component of this Example 2 was made as follows. We mixed:

400.0 grams distilled water  
0.1 gram "TRITON X-114"  
0.1 gram antifoam agent.

"TRITON X-114" is a surface-active agent having emulsifying, wetting and dispersing properties. It includes alkylaryl polyether alcohols, sulfonates and sulfates. It is a non-ionic type and is manufactured by Rohm & Haas Company. Its hydrophilic-lipophilic balance (HLB value) is 12.4. Its molecular weight is approximately 536 and its density is 8.8. Any appropriate antifoam agent can be used. One is manufactured by Dow, Corning and is a silicone defoamer that is effective in very low concentrations. Another silicone-base antifoaming agent is manufactured by Laurel Soap Manufacturing Company.

It is to be understood that any appropriate emulsifying agent may be employed to give stability to the emulsion. The emulsifying agent, however, must always be more

soluble in or better wetted by the continuous or lipide phase than the disperse or aqueous phase. The surface-active emulsifying agents are neither completely hydrophilic nor completely lipophilic. Another emulsifying agent is composed of polyoxyalkylene derivatives of sorbitane fatty acids.

The emulsion of Example 2 is manufactured by emulsifying 100 grams of "ISOPAR G" with 250 grams of the organosol of Example 2 together with the water component of Example 2 just described. The emulsification may take place in a homogenizer, a colloid mill, or in a sonic or ultrasonic emulsifying apparatus. We have found that a colloid mill does not give as good an emulsifying action as an ultrasonic emulsifier. The better the dispersion, the higher may be the water-to-adhesive toner ratio. With a good emulsifying action, the "ISOPAR G" which is now used in the formulation may be materially reduced or eliminated completely, so that we will emulsify a pigmented solution of a high molecular weight resin directly with water, the latter being in the disperse phase.

The emulsion of Example 2 develops a latent electrostatic image on a negatively charged photoconductor. The emulsion is stable and will not conduct electricity. Since the photoconductive surface is hydrophobic, the droplets of water released during development are readily blown away by an air knife.

It will be observed that we are emulsifying the liquid developer described in our co-pending application, Ser. No. 155,108, with water and that the lipide phase is a suspension or emulsion of an organosol in a light hydrocarbon diluent. Accordingly, we have a complex system in which the lipide phase is a suspension of an organosol.

We are still conducting experiments in making emulsions with the object of reducing the isoparaffin or diluent component since this is what must be evaporated after the electrostatic image is developed. It will be seen, however, that we have greatly reduced the amount of isoparaffinic hydrocarbons which must be evaporated by our aqueous emulsion.

#### EXAMPLE 3

To the materials we mixed in Example 2 we add a release agent such as polyethylene wax, polyvinyl stearate, polyvinyl chloride resin, silicon resin, or reactive silicon fluid, in amounts varying between 4 grams and 14 grams by weight. The release agents are co-deposited with the organosol during development and assist in the transfer of the developed image from the surface of the photoconductor to the paper. These release agents are described in our co-pending application,<sup>1</sup> Ser. No. 269,054, mentioned above. The use of a release agent not only assists in the complete transfer of the developed tacky image, but aids in keeping the photoconductive surface clean for a longer period of time. Furthermore, in the event the photoconductive surface becomes soiled, it is more readily cleaned when release agents are used.

It will be seen that we have accomplished the objects of our invention. We have provided an aqueous emulsion in which the organosol is in the continuous phase and in which water is in the disperse phase so that, upon development of a latent electrostatic image, water instead of a light hydrocarbon liquid is released. This substantially reduces the pollution of the atmosphere which would be caused by the evaporation of a light hydrocarbon diluent as a carrier for the organosol toner.

The use of an emulsifying agent provides a stable emulsion, and the advantage of a release agent in the continuous phase assists in the complete transfer of the tacky developed image from the photoconductor to the paper or other sheet material.

It will be understood that certain features and subcombinations are of utility and may be employed without reference to other features and subcombinations. This is

contemplated by and is within the scope of our claims. It is further obvious that various changes may be made in details within the scope of our claims without departing from the spirit of our invention. It is, therefore, to be understood that our invention is not to be limited to the specific details shown and described.

Having thus described our invention, what we claim is:

1. A developing emulsion for use in developing a latent electrostatic image including in combination a tacky organosol lipide phase comprising the following by weight:

|                               | Percent   |
|-------------------------------|-----------|
| High molecular weight polymer | 3.5-5.5   |
| Light hydrocarbon liquid      | 32.0-52.0 |
| Pigment                       | 0.5-1.5   |

in which said light hydrocarbon liquid includes about 90% isoparaffinic hydrocarbons and about 10% aromatic hydrocarbons, and a disperse aqueous phase comprising the following by weight:

|                                  | Percent   |
|----------------------------------|-----------|
| Water                            | 43.0-64.0 |
| Surface-active emulsifying agent | 0.01-0.15 |
| Antifoam agent                   | 0.01-0.15 |

said high molecular weight polymer being dissolved in said aromatic hydrocarbon liquid.

2. A developing emulsion as in Claim 1 in which the lipide phase carries between 0.5% and 1.0% of a release agent.

3. A developing emulsion for use in developing a latent electrostatic image including in combination a continuous

phase comprising a tacky high molecular weight polymeric resin dissolved in an aromatic hydrocarbon solvent dispersed in a light isoparaffinic hydrocarbon liquid said light isoparaffinic hydrocarbon liquid comprises about 90% of the hydrocarbon liquids in the developing emulsion together with a pigment, and a discontinuous aqueous phase comprising water, a minor amount of a surface-active stabilizing agent more soluble in the continuous phase than in water, and a minor amount of an antifoam agent.

4. A developing emulsion as in Claim 3 in which the lipide phase carries a minor amount of a release agent.

#### References Cited

##### UNITED STATES PATENTS

|    |           |         |                 |          |
|----|-----------|---------|-----------------|----------|
| 15 | 3,156,531 | 11/1964 | Fauser et al.   | 252-62.1 |
|    | 3,001,888 | 9/1961  | Metcalfe et al. | 252-62.1 |
|    | 2,637,621 | 5/1953  | Auer            | 8-62     |
|    | 2,594,899 | 4/1952  | Fordemwalt      | 8-62     |
|    | 2,383,937 | 9/1945  | Kienle et al.   | 8-62     |
| 20 | 2,323,871 | 7/1943  | Kienle et al.   | 8-62     |
|    | 2,307,097 | 1/1943  | Anderson        | 8-62     |
|    | 3,301,698 | 1/1967  | Fauser et al.   | 252-62.1 |

#### OTHER REFERENCES

25 "Water as an Electrostatic Toner," *Product Licensing Index*, March, 1972, pp. 46-47.

RONALD H. SMITH, Primary Examiner

30 J. P. BRAMMER, Assistant Examiner